

## 1

3,475,237

BORON FUEL-SALT SMOKE-PRODUCING  
COMPOSITIONS

George A. Lane and William A. Smith, Midland, and  
Ralph B. Van Wert, Essexville, Mich., assignors to  
The Dow Chemical Company, Midland, Mich., a cor-  
poration of Delaware  
No Drawing. Filed July 1, 1968, Ser. No. 741,244  
Int. Cl. C06d 3/00; C06b 11/00

U.S. Cl. 149—22

4 Claims

creases as particle size decreases. Generally, the particle size of the materials ranges from about 5 to about 400 microns.

The pyrotechnic smoke-producing compounds of the present invention can be fabricated by admixing the particulate boron-containing fuel and particulate oxidizer until a substantially homogeneous blend is obtained. The so-homogenized blend is enclosed in a suitable container and compacted by conventional means to about 2000 p.s.i. The resulting compressed grain is initiated with commonly employed ignition system such as a fuse.

## 2

## PREFERRED EMBODIMENTS

A preferred embodiment of the present invention comprises a pyrotechnic smoke producing munition comprising on a weight basis of from about 30 to about 70 percent of elemental boron, and from about 70 to about 30 percent of a member selected from the group consisting of alkali metal- and ammonium nitrates, -chlorates, -perchlorates and mixtures thereof.

Very good smoke production can be obtained where about 40 percent by weight of the munition is substantially anhydrous lithium perchlorate or sodium perchlorate and the balance is boron.

Another preferred embodiment of the present invention is the smoke-producing munition consisting by weight of from about 25 to about 70 percent boron carbide, and from about 75 to about 30 percent of an inorganic oxidizer selected from the group consisting of alkali metal and ammonium nitrates, chlorates and perchlorates. Most preferably, the oxidizer will be substantially anhydrous lithium perchlorate.

Still another preferred embodiment is the pyrotechnic composition consisting by weight of from about 25 to about 65 percent of particulate decaborane fuel and from about 75 to about 35 percent of a member selected from the group consisting of guanidine nitrate, anhydrous lithium perchlorate, and mixtures thereof, as oxidizer.

To fabricate the pyrotechnic munitions described directly hereinabove, the particles of oxidizer and fuel are admixed until substantially homogeneous, placed in a heat resistant container and compacted by commonly employed means to about 2000 p.s.i. and the resulting pressed grain is initiated with a commonly employed ignition fuse.

The following examples are set forth to illustrate the present invention and are not intended as limits thereto.

## Example 1

About 6 grams of particulate elemental boron and about 4 grams of substantially anhydrous particulate lithium perchlorate ( $\text{LiClO}_4$ ) were admixed until substantially homogeneous. The particle size of the materials employed ranged from about 5 to about 200 microns. The so-homogenized mixture was placed in a steel cylinder about  $1\frac{1}{2}$  inches in diameter and about 1 inch in height, and compacted to about 2000 p.s.i. using a standard hydraulic press. The resulting pressed grain munition was initiated with a thermalite Ignitacord brand fuse.

Upon ignition, the burning time, aerosol yield

$$\text{Aerosol yield (percent)} = \frac{\text{Agent in Aerosol Form} \times 100}{\text{Total Weight Composition}}$$

and efficiency,

$$\text{Efficiency (percent)} = \frac{\text{Agent in Aerosol Form} \times 100}{\text{Agent in Composition}}$$

were measured. Additionally, the total obscuring power (TOP) of each munition was measured in terms of area obscured per pound of munition employed.

Upon ignition, the efficiency of dissemination was about

## ABSTRACT OF THE DISCLOSURE

The present disclosure relates to smoke-producing pyrotechnic pressed grain compositions consisting of a 15 boron-containing fuel and an organic or inorganic oxidizer.

## BACKGROUND OF INVENTION

In wartime the armed forces frequently find it necessary to employ smoke screens to shield troop movements from the enemy.

Presently, the active ingredients in smoke-screening devices are white phosphorus, titanium tetrachloride, chlorosulphonic acid, sulfur trioxide, zinc chloride, and oils. All of these agents, with the exception of the oils, react with the atmosphere to produce smokes which are both corrosive and toxic. Oil smokes, while non-toxic and non-corrosive demonstrate relatively poor obscuring power.

An object of the present invention is to produce pyrotechnic compositions which can be ignited to yield voluminous and dense screening smokes which are non-corrosive and relative non-toxic.

## SUMMARY OF THE INVENTION

The pyrotechnic smoke producing composition of the present invention consists by weight of from about 25 percent to about 75 percent of a boron-containing fuel compound with the balance being an organic or inorganic oxidizer.

The boron-containing fuel is generally a member selected from the class consisting of elemental boron, boron carbide, boranes containing from about 5 to about 10 boron atoms per molecule, and mixtures thereof. Additionally, boron silicides and other compounds consisting essentially of boron and silicon can be employed as fuels in the present invention.

Methyl borate and trimethoxyboroxine can also be employed in the present invention as boron-containing fuel compounds. Because of the liquid nature of methyl borate and trimethoxyboroxine, it is desirable to disperse these compounds within particulate inert absorbent carrier compounds such as expanded clays, alumina, and porous silicates. Said particulate carrier compounds containing the boron fuel can be admixed with the particulate oxidizer homogeneous, and the so-homogenized blend can be placed in a suitable container and compacted under pressure. The resulting pressed grain munition can be initiated with a commonly employed ignition system.

Generally the oxidizer employed is a member selected from the group consisting of the alkali metal- or ammonium nitrates, -chlorates and -perchlorates, guanidine nitrate, and mixtures thereof. Preferably, where an inorganic oxidizer is employed, said oxidizer will be substantially anhydrous, although hydrated inorganic oxidizers are operable in the present invention.

Both oxidizer and fuel should be in a particulate form and while particles of almost any size can be employed in the present invention, smoke production efficiency in-

55 percent, the yield was about 100 percent, and the obscuring power was about 5500 ft.<sup>2</sup> obscured per pound of munition employed.

It should be noted that smoke production and obscuring power increase as the relative humidity increases. The above experiment was carried out at a relative humidity of about 55 percent.

## Example 5

Employing a process of fabrication substantially similar to the process set forth in Example 1, various samples were prepared and tested to compare obscuring power with the obscuring power produced by a standard titanium chloride composition. The test results are set forth in Table V.

TABLE V

| Run No.: | Munition Composition (parts by weight)                | Efficiency, percent <sup>1</sup> | Yield, percent <sup>2</sup> | TOP, <sup>3</sup> ft. <sup>2</sup> /lb. | Burning Time, sec. |
|----------|-------------------------------------------------------|----------------------------------|-----------------------------|-----------------------------------------|--------------------|
| 1.....   | 60 Boron/50 LiClO <sub>4</sub> .....                  | 55.0                             | ~100                        | 6,000                                   | 1                  |
| 2.....   | 65 B <sub>10</sub> H <sub>14</sub> /35 guanidine..... | 60                               | ~100                        | 4,800                                   | .....              |
| 3.....   | TiCl <sub>4</sub> (control).....                      |                                  |                             | 4,100                                   | .....              |

<sup>1</sup> Efficiency, percent conversion of fuel to smoke.

<sup>2</sup> Yield, percent of smoke generated from a given weight of munition.

<sup>3</sup> TOP, total obscuring power, ft.<sup>2</sup>/lb.

## Example 2

Employing a process substantially similar to the process described in Example 1, other samples were prepared wherein the relative amounts of boron fuel and lithium perchlorate oxidizer were varied. Upon ignition these samples yielded the data set forth in Table I.

TABLE I

| Run No.: | Composition        |                                  |                                                   |
|----------|--------------------|----------------------------------|---------------------------------------------------|
|          | Boron, wt. percent | LiClO <sub>4</sub> , wt. percent | Total Obscuring Power (TOP) ft. <sup>2</sup> /lb. |
| 1.....   | 30                 | 70                               | 4,790                                             |
| 2.....   | 40                 | 60                               | 4,370                                             |
| 3.....   | 50                 | 50                               | 5,500                                             |
| 4.....   | 60                 | 40                               | 5,680                                             |
| 5.....   | 70                 | 30                               | 4,970                                             |

From Table I it can be seen that for this fuel and oxidizer optimum obscuring power is obtained when the composition consists by weight of about 60 percent elemental boron and about 40 percent lithium perchlorate. The particle size of fuel and oxidizer employed ranged from about 5 to about 200 microns.

## Example 3

Employing substantially the process set forth in Example 1, a munition grain consisting of about 55 grams of elemental boron and about 45 grams of NaClO<sub>4</sub> was prepared and ignited. The total obscuring power was about 5,900 ft.<sup>2</sup>/lb. of munition employed. The relative humidity at the time of ignition was about 65 percent.

## Example 4

Employing substantially the process set forth in Example 1, pressed grains consisting of boron carbide (B<sub>4</sub>C) and anhydrous lithium perchlorate were prepared and ignited to yield the data set forth in Table II. The particle size of the carbide and perchlorate materials ranged from about 5 to about 200 microns. The relative humidity was about 75 percent.

TABLE II

| Run No.: | Composition                   |                                  |                                        |
|----------|-------------------------------|----------------------------------|----------------------------------------|
|          | B <sub>4</sub> C, wt. Percent | LiClO <sub>4</sub> , wt. Percent | Obscuring Power, ft. <sup>2</sup> /lb. |
| 1.....   | 25                            | 75                               | 2,800                                  |
| 2.....   | 30                            | 70                               | 4,320                                  |
| 3.....   | 35                            | 65                               | 2,840                                  |
| 4.....   | 50                            | 50                               | 2,960                                  |
| 5.....   | 70                            | 30                               | 1,860                                  |

From Table II it can be seen that optimum obscuring power is obtained when this munition consists by weight of about 30 percent boron carbide and about 70 percent lithium perchlorate.

From Table V it can be seen that compositions of the present invention produce obscuring smoke screens substantially equivalent to those produced by titanium chloride.

The examples set forth directly hereinabove are intended solely as illustrations and not as limitations upon the present invention, for said invention is limited only 25 by the appended claims.

We claim:

1. A pyrotechnic smoke-producing composition consisting essentially by weight of from about 25 to about 75 percent of a fuel selected from the group consisting of elemental boron, borane compounds containing from about 5 to about 10 carbon atoms per molecule, methyl borate, trimethoxyboroxine, and mixtures thereof, and from about 30 to 70 percent of a particulate oxidizer selected from the group consisting of alkali metal- and ammonium-perchlorates, -chlorates, -nitrates, and -nitrites, guanidine nitrate, and mixtures thereof, as oxidizer.

2. A pyrotechnic smoke-producing composition consisting essentially of by weight from about 30 to about 70 percent particulate elemental boron as fuel, and from about 70 to about 30 percent of an oxidizer selected from the group consisting of alkali metal- or ammonium perchlorates, -chlorates, -nitrates and mixtures thereof.

3. The composition as defined in claim 2 wherein about 40 percent by weight is an oxidizer member selected from the group consisting of substantially anhydrous lithium perchlorate and sodium perchlorate, and the balance is boron.

4. The composition defined in claim 1 wherein from about 25 to about 65 percent of decaborane as fuel compound, and from about 80 to about 35 percent of an oxidizer member selected from the group consisting of guanidine nitrate and anhydrous lithium perchlorate.

## References Cited

## UNITED STATES PATENTS

|           |         |                 |          |
|-----------|---------|-----------------|----------|
| 3,009,800 | 11/1961 | Swimmer         | 149—22 X |
| 2,796,339 | 6/1957  | Jackson         | 149—22   |
| 3,070,472 | 12/1962 | Drummond        | 149—22   |
| 3,122,462 | 2/1964  | Kaufman         | 149—22 X |
| 3,126,305 | 3/1964  | Armstrong       | 149—22 X |
| 3,130,097 | 4/1964  | Drummond        | 149—22   |
| 3,135,635 | 6/1964  | Logan et al.    | 149—22   |
| 3,150,019 | 9/1964  | Logan et al.    | 149—22   |
| 3,238,076 | 3/1966  | Taylor et al.   | 149—22   |
| 3,240,640 | 3/1966  | Ives            | 149—22 X |
| 3,247,034 | 4/1966  | D'Alelio        | 149—22 X |
| 3,257,801 | 6/1966  | Martinez et al. | 149—22 X |

CARL D. QUARFORTH, Primary Examiner

S. J. LECHERT, Assistant Examiner

U.S. CL. X.R.

149—38, 40, 41, 42, 43, 46, 47, 61, 62, 70, 75, 76, 77, 78,  
75 83, 85